

1  
2,851,355

PROCESS FOR THE PREPARATION OF  
SEMI-CELLULOSE

Ernst Battenberg, Mannheim-Waldhof, and Heinz Haas,  
Weinheim, Bergstrasse, Germany, assignors to Zell-  
stofffabrik Waldhof, Mannheim-Waldhof, Germany, a  
German joint-stock company

No Drawing. Application November 15, 1951

Serial No. 256,593

Claims priority, application Germany February 28, 1951  
3 Claims. (Cl. 92—11)

The invention relates to a process for the preparation of semi-chemical cellulose pulp by the treatment of cellulose containing raw materials with an acidified bisulfite cooking solution at a pH of about 3.5–6, containing from 1.4–3.0% of  $\text{SO}_2$ , at cooking temperatures between 115° and 140° C., to effect thereby a mild decomposition of the cellulose starting material, which only slightly attacks the cellulose and hemi-cellulose and which removes to a great extent the lignin binding the cellulose fibers in the middle lamellae of the starting cellulose material to produce cellulose fiber bundles which adhere so solidly that they require additional mechanical defibrillation to provide separate individual fibers in the product.

As starting materials cellulose containing plant products may be employed which are obtained from any convenient source such as deciduous or foliaceous trees, coniferous trees, soft woods, hard woods, annual plants, and plant wastes such as bagasse, palm oil fibers and alfalfa fibers.

The hard woods may be hardwoods such as: Aspen (*Populus tremuloides* and *deltoides*)—Large-toothed aspen (*Populus grandidentata*)—Beech (*Fagus grandifolia* *Antropuncea* and *sylvatica*) Red alder (*Alnus rubra*)—Sycamore (*Platanus occidentalis*)—Tupelo gum (*Nyssa aquatica*)—Black gum (*Nyssa sylvatica*) Red gum (*Liquidamber styraciflua*) Red maple (*Acer rubrum*)—White maple (*Acer saccharinum*)—Buckeye (*Aesculus glabra*)—Cucumber magnolia (*Magnolia acuminata*)—Yellow poplar (*Liriodendron tulipifera*)—American elm (*Ulmus americana*)—Basswood (*Tilia americana*)—Paper birch (*Betula papyrifera*)—Yellow birch (*Betula lutea*)—Chestnut (*Castanea dentata*).

Yearly plants such as: Esparto (*Stipa tenacissima*)—Corn stalks (*zea mays*)—Sorgho (sorghum Lum)—Am-pelodesma Tenax—Papyrus (*Cyperus papyrus*)—Straw (rice, barley, wheat)—Daffodil (*Asphodelus ramousus*) are useful.

Stem-plants such as: Hemp stem (*Cannabis sativa*), manila stem (*Musa textilis*), jute stem (*Corchorus capsularis*) paper mulberry (*Broussonetia papyrifera*), Agave (*Agave rigidula*), sisal, flax straw (*Linum usitatissimum*), cane (*arundo donax* and *Phragmites*), Ghinda (*Calotropis procera*), cotton stems (*Gossypium*), sugar cane bagasse, bamboo (*Bambusa arundinacea*) are useful.

Plant wastes of special plants as: palm oil (*Elaeis guineensis*) fibers, and other fibers having same physico-chemical composition, Cecropia may be used.

Wood waste such as saw mill waste, ply-wood waste, matches waste may be used.

The semi-chemical pulp in the process of the application is obtained in yields of approximately 70–80% relative to the cellulose content of the starting material as contrasted with the yields of approximately 45% realized in the normal pulping process.

In addition to the advantage of obtaining higher yields of cellulose by the process of the invention, the improved strength characteristics of the semi-chemical pulp product, the lower lignin content of the product and the very high

hemi-cellulose content of the semi-chemical pulp product provide unusual beneficial advantages over the semi-chemical processes heretofore known. The process herein requires smaller quantities of treating chemicals and therefore permits the manufacture at lower costs as compared with the semi-chemical pulping processes in the prior art. Because of the greater hemi-cellulose content obtained in the process of the application, the semi-chemical pulp product offers excellent bleaching qualities to provide a bleached pulp of brighter color and relatively unimpaired strength.

Numerous semi-chemical processes have heretofore become known, among which particular attention has been paid to an alkaline process, preferably with caustic soda, a neutral sulfite process with  $\text{Na}_2\text{SO}_3$  in presence of sodium bicarbonate, developed more especially in the United States, and an acid process with bisulfite-cooking acids.

The alkaline semi-chemical decomposition processes consist in using the cooking liquors which are conventional for the sulfite or soda processes, in some cases with addition of accumulated waste liquors, which may be of lesser concentration, and conducting the cooking in such manner at temperatures of 160–170° C. and at a pH above 7 that the obtained semi-chemical fiber bundles are capable of mechanical defibrillation.

The alkaline decomposition process for the preparation of semi-chemical cellulose pulp is required to conduct the cooking of the lignin containing cellulose starting material to a point where the fibers are easily separated. Such cooking under the alkaline conditions present in the cooking liquor and at the temperature employed causes a far greater loss of hemi-cellulose in the semi-chemical pulp product and at the same time provides lower yields as increasing amounts of lignin are removed. This results in poorer strength characteristics in the product.

The neutral sulfite process is carried out with  $\text{SO}_2$ -concentrations of 3–5%, all the sulfurous acid being bound to alkali so that generally an excess of alkali is present, this process being therefore carried out at pH-values above 7.0 and at temperatures of 160–170°.

In the neutral sulfate process of alkali sulfate semi-chemical cellulose pulp decomposition the cellulose decomposition is greater, but there is a smaller dissolving-out of hemi-celluloses and extracted substances, and more lignin than obtained in the alkaline process.

In the alkaline sulfate process, the cellulose decomposition, as compared to the other processes, is lower, the fraction of dissolved-out hemi-celluloses and extracted substances is higher, and the lignin solution is smaller.

In the acid semi-chemical cellulose pulp process, e. g. with sodium bisulfite, which because of its high requirement for chemical reagents is less in vogue today, use is made of a decomposition liquid with 3.5–6% and more of  $\text{SO}_2$  at temperatures of the conventional bisulfite process between 120–140°. 50% of the sodium-bound sulfurous acid is in the form of  $\text{NaHSO}_3$ , so that there is a pH-value of about 2.0. A comparison of the constituents in alpha-celluloses, hemi-celluloses, lignin and extracted substances, removed in these decomposition processes shows, for equal yields, the following:

In the acid process with bisulfite-cooking acids, the cellulose decomposition is somewhat less than in the neutral sulfite process, more hemi-celluloses are retained and the fraction of dissolved lignins is higher. In addition to the more favorable composition, this semi-chemical cellulose pulp excels also in its higher yield and lighter color; in addition, its bleachability is better than in the materials obtained according to alkaline or neutral processes.

In the production of semi-chemical pulp from annual

plants, Aronowsky et al., "Agricultural Residue Pulps Comparison of Pulping Processes Paper Trade Journal, vol. 126, N. 26 (1949)" concluded that the acid pulping processes produced relatively weak and brittle pulps from straw. It was apparent that these processes were unsuitable for producing strong and satisfactory pulps from agricultural residues of high silica content. These workers using conventional bisulfite liquor (5%  $\text{SO}_2$ ) at 140° obtained a yield of 40% raw pulp and which corresponded to a consumption of 200 kg. of sulphur per ton of air-dried pulp.

The neutral sulfite process, which is more expensive than the process of the invention because of its greater consumption of chemicals, has nevertheless been widely adopted in the United States because it was not heretofore possible according to known acid bisulfite processes to obtain semi-chemical cellulose pulp with sufficient strength properties, as compared to those from the neutral sulfite process. This neutral sulfite process represents a compromise between the high yield of the acid bisulfite process and the good strength properties of the alkaline process.

The following Table I sets forth yield data with the usual sulfite cellulose processes obtained from deciduous wood, and in which according to Professor Chidester, the deciduous starting wood contains approximately 50% cellulose, approximately 25% hemi-cellulose, approximately 21% lignin and approximately 4% residue in the form of extract substances.

uring Methods: Alpha-cellulose T201  $m$ -46, hemi-cellulose T223  $m$ -48. Lignin was determined according to D. M. Halse (Paper Journal 10, 121, 1926).

TABLE I

|                       | Alkali, percent | Neutral, percent | Acid, percent | Applica-<br>tion process,<br>percent |
|-----------------------|-----------------|------------------|---------------|--------------------------------------|
| Alpha cellulose.....  | 46.0            | 44.0             | 44.3          | 44.2                                 |
| Hemi-cellulose.....   | 13.5            | 15.0             | 18.2          | 16.5                                 |
| Lignin.....           | 14.5            | 13.0             | 10.5          | 11.8                                 |
| Other components..... | 1.0             | 2.0              | 2.0           | 2.0                                  |

Table I indicates that the acid semi-chemical pulps have the lowest lignin contents and at the same time the highest semi-cellulose contents.

Table II, below, summarizes the operating conditions of the alkali semi-chemical pulp process, the neutral sulfite process, the acid sulfite process of the prior art and of the process of the invention.

The values indicated in Table II below encompass deciduous woods and coniferous woods of the most valuable type, the individual data corresponding to the particular wood being used. The yield in the normal bisulfite process usually amounts to about 40-50% and for all semi-chemical cellulose pulp decomposition processes to about 70-85%. These yields are not determined by the process itself, but are dependent upon particular selected conditions.

TABLE II

## Process of manufacturing paper-pulps

| Process                                         | Amount of $\text{SO}_2$ in Liquor, percent                                  | Proportion, wood: liquor | pH by cooking, beginning                                                       | Temperature by cooking, °C. | $H_1$ =Impregnation time in hours: $H_2$ =cooking time in hours |
|-------------------------------------------------|-----------------------------------------------------------------------------|--------------------------|--------------------------------------------------------------------------------|-----------------------------|-----------------------------------------------------------------|
| Conventional bisulfite-process.                 | 4-6%.....                                                                   | 1:4.5                    | 1.2-2.0.....                                                                   | over 125                    | $H_1=2-5$ or 6-8;<br>$H_2=5-8$ or 16.<br>$H_2=ca. 6-7.$         |
| Acid process of semi-chemical pulps.            | 3.5-6%.....                                                                 |                          | 2.0-3.0.....                                                                   | 120-140                     |                                                                 |
| Neutral sulfite process of semi-chemical pulps. | 3-5%.....                                                                   | 1:4-5                    | 6.0-8.0.....                                                                   | 140-170                     | $H_1=1-2$ ; $H_2=4-10.$                                         |
| Application process for semi-chemical pulps.    | 1.4-3.0% (with leaf wood 1.4-1.8% coniferous trees to 2.8% straw ca. 1.4%). | 1:4-4.5                  | 3.5-6.0 (with Calcium pH=4.5, Temp. 125-130°; with Mg pH=5-6, Temp. ca. 140°). | 115-140                     | $H_1=3-7$ ; $H_2=3-5.$                                          |

If deciduous wood, e. g. aspen wood, is decomposed into semi-chemical cellulose pulp according to the known process under alkaline, neutral and acid conditions, and then according to the process of the application, in each case to a 75% wood yield, there obtain the aforementioned total ingredients in the amounts as set forth in Table I.

It is to be noted that, of these values, the cellulose and semi-chemical cellulose pulp determinations were obtained according to the following TAPPI Standard Meas-

In the following Table III the manufacturing costs, calculated from the costs of the chemicals and the total production costs such as steam, water, labor, including collateral costs of unbleached semi-chemical cellulose pulp prepared according to the known process are compared with the corresponding costs for semi-chemical cellulose pulp prepared according to the process of the present invention, and that for deciduous woods (beech). The values relate to one ton of absolutely dry (atro) semi-chemical cellulose pulp, at a 75% yield.

TABLE III

| Material consumption, consumption in power, labor, incidental costs etc. (Production costs) | For known semi-cellulose processes (neutral sulfite processes) in the United States and other countries |        |                 | For the processes according to the invention              |        |
|---------------------------------------------------------------------------------------------|---------------------------------------------------------------------------------------------------------|--------|-----------------|-----------------------------------------------------------|--------|
|                                                                                             | Required quantities in kg. per ton of semi-cellulose, kg.                                               | Costs  |                 | Required quantities in kg. per ton of semi-cellulose, kg. | Costs  |
|                                                                                             |                                                                                                         | DM     | \$(DM 4.20=\$1) |                                                           |        |
| Wood (Beech).....                                                                           | 1,335                                                                                                   | 142.09 | 33.83           | 1,335                                                     | 142.09 |
| Sulphur.....                                                                                | 70                                                                                                      | 9.15   | 2.18            | 43                                                        | 5.65   |
| Soda.....                                                                                   | 350                                                                                                     | 42.00  | 10.00           |                                                           |        |
| NaOH.....                                                                                   |                                                                                                         |        |                 | 25                                                        | 0.64   |
| Polysphosphate.....                                                                         |                                                                                                         |        |                 | 0.3                                                       | 0.21   |
| Lime.....                                                                                   |                                                                                                         |        |                 | 68                                                        | 1.10   |
| Production Costs.....                                                                       |                                                                                                         | 114.55 | 27.27           |                                                           | 102.53 |
|                                                                                             |                                                                                                         | 307.79 | 73.28           |                                                           | 254.97 |
|                                                                                             |                                                                                                         |        |                 |                                                           | 60.70  |

It can be seen from Table III that the costs of the new process, relative to the known process, are approximately 17.5% less than the known processes. This represents a very substantial decrease in cost of production.

An object of the invention is the decomposition of cellulose containing starting materials with a bisulfite cooking liquor containing from about 1.4-3% of  $\text{SO}_2$  at a pH of from 3.5-6 and a reaction temperature of about 115-140° C. to obtain thereby a removal of the lignin from the cellulose fibers in the middle lamellae of the starting material and to provide a product which can be readily mechanically defibrillated.

A further object of the invention is the preparation of semi-chemical cellulose pulp by the treatment of cellulose containing raw material with a bisulfite solution containing 1.4-3%  $\text{SO}_2$  in the bisulfite liquor, at a pH of 3.5-6, and a reaction temperature of about 115-140° C., wherein in the cooking liquor is buffered by polyphosphates, metaphosphates, hexametaphosphates, imidoacetic acid, nitrilotriacetic acid, etc. together with a base such as sodium hydroxide, sodium carbonate, potassium hydroxide, calcium hydroxide, magnesium oxide, aluminum hydroxide, ammonia and alkaline organic amines. Polyphosphates of general formula  $(\text{Na}_{n+2})\text{P}_n(\text{O}_{3n+1})$  are used, especially those wherein  $n=3$  or 4. Also suitable are metaphosphates of the general formula  $(\text{KPO}_3)_x$ , hexametaphosphates of the foregoing formula with  $x=6$ , imino-diacetic acid of the formula  $\text{HN}(\text{CH}_2\text{CO}_2\text{H})_2$ , nitrilotriacetic acid of the formula  $\text{N}(\text{CH}_2\text{CO}_2\text{H})_3$ , ethylene diamine tetraacetic acid of the formula  $\text{C}_2\text{H}_4\text{N}_2(\text{CH}_2\text{CO}_2\text{H})_4$ , lower aliphatic amines, etc.

Other and further objects of the present invention will appear from the more detailed description set forth below, it being understood that such more detailed description is given by way of illustration and explanation only and not by way of limitation.

According to the invention, the semi-chemical cellulose pulp decomposition takes place in aqueous solution of  $\text{SO}_2$  and of a base, such as bases derived from calcium, magnesium, sodium, ammonia, aluminum, etc., under reaction conditions which may broadly be considered as between those of the known acid bisulfite process and the neutral sulfite process. This requires that the pH-value of the cooking acid, as compared with the pH-values of the acid process, be higher and that the  $\text{SO}_2$ -content as well as the reaction temperatures be lower, relative to the neutral sulfite process. The new reaction conditions are explained in greater detail in the following.

The increase in pH-value of an alkali, e. g. calcium bisulfite-cooking acid, means that the quantity of free  $\text{SO}_2$  is greatly reduced and the possibility of a hydrolytic decomposition of the cellulose decreased. The reaction conditions prevailing in the neutral sulfite process are thus more nearly approached. With the individual cations, this is possible only to a certain extent, since a certain amount of free  $\text{SO}_2$  has to be present if the bisulfite is to remain in solution. According to the invention, the increase in pH-value can take place after buffering e. g. with  $\text{NaOH}$ ,  $\text{KOH}$ ,  $\text{NH}_3$ , amines, etc.

In order not to exceed the solubility of the sulfite, e. g. the solubility of the  $\text{CaSO}_3$ , with calcium as the base, the buffering agent has to be added in the presence of a complex builder. Complex builders are e. g. polyphosphates, such a Calgon (a water-softening agent consisting essentially of sodium hexametaphosphate), tripolyphosphates, sodium polyphosphate, sodium pyrophosphate, acid sodium pyrophosphate, etc., nitrilotriacetic acid or imido-diacetic acid.

It is necessary to raise the pH-value to 3.5-6. When using bisulfites of other cations, e. g. of magnesium, it is possible by the addition of  $\text{NaOH}$  only to prepare a substantially neutral cooking liquid. It has been found that the acidity during the cooking exerts an important influence on the strength properties and gives best values with the above-indicated starting value.

Since, in the semi-chemical cellulose pulp decomposition of the invention, only a partial removal of the lignin, specifically, that of the middle lamellae, is achieved, the process employs a smaller quantity of  $\text{SO}_2$  relative to the normal bisulfite decomposition. About 45% of the lignin present is sulfonated and removed as lignin sulfonic acid or its salts in the process of the invention.

In order to realize a sufficient sulfonation and hydrolytic splitting of the sulfonic acid, when the buffered acid has a pH=3.5-6, use is made according to the invention of a cooking acid with a 1.4-3% total  $-\text{SO}_2-$  content, depending upon the starting material. With foliaceous trees, especially beech trees, which strongly reduce the pH-value during the cooking by the splitting off of organic acids, the use of a cooking acid with 1.4-1.8%  $\text{SO}_2$  is favorable, while with coniferous trees, which contain more lignin, higher  $\text{SO}_2$ -concentrations up to 2.8% and higher are necessary. With annual plants, e. g. straw,  $\text{SO}_2$ -concentrations of about 1.4% suffice.

10 In the acid decomposition process of the invention the reaction temperature exerts an essential influence on the hydrolysis of the hemi-celluloses and of the cellulose present. Although, in an alkaline decomposition process as well as in a neutral sulfite semi-chemical cellulose pulp process, an increase in temperature appreciably influences the reaction speed, in the acid process a temperature increase is prejudicial to the fiber strength properties because of an increase in the hydrolysis. Temperatures can be adopted for various degrees of acidity, below 15 which temperatures, no appreciable impairment of fiber strength takes place. For a process carried out according to the invention, e. g. with calcium as the base, at a pH=4.5, the temperatures may amount to about 125-130°; for a magnesium bisulfite solution with a pH=5-6, temperatures of about 140° are indicated.

20 The ratio of wood to liquor is, according to the invention, about 1 : 4-5. The time of impregnation, i. e. of the first part of the cooking, amounts to about 3-7 hours, at temperatures which, compared to the end temperatures of the cooking proper, are about 20-30° C. lower than the end temperatures. The cooking proper lasts 3-5 hours, the temperature being preferably raised in one stage.

25 According to the new semi-chemical cellulose pulp decomposition process with a cooking acid at a pH=4-6 and a total  $-\text{SO}_2-$  content of 1.4-3%, fibrous materials are obtained in a yield of 70-85% (with certainty) after mechanical treatment without bleaching. The amount of cellulose and hemi-celluloses obtained fluctuates only 30 slightly, so that the yield depends essentially upon the amount of removed lignin.

35 Notwithstanding the high lignin content of 10-15% the product is well bleachable by the usual bleaching processes employing a total quantity of about 10-14% chlorine, the achieved degree of whiteness being between 55 85 and 90% units on the GE scale. The bleachability is essentially better than that obtained according to the sulfite process, for which the bleaching degree is at most 85% on GE scale.

40 The yield in cellulose product rich in bleached semi-chemical cellulose pulp is 60-65%, relative to the wood, which yield also is greater than the yield of cellulose according to the neutral sulfite process.

45 The strength properties and bleachability of the semi-chemical cellulose pulp are considerably improved compared with the corresponding cellulose of the usual processes. Semi-chemical cellulose pulps which are cooked to obtain yields of 75-80%, have the best strength values, while with higher yields, i. e., with increasing lignin content, an increasing brittleness and a decrease in strength properties, especially in folding number, becomes perceptible. It has been found that the strength properties of the semi-chemical cellulose pulp prepared according to the process of the present invention are equal to those obtained from the material decomposed according to the 50 75

neutral sulfite process; a particular advantage relative to this process of the invention is the lower consumption of chemicals and thus the lower manufacturing costs. A further improvement of the properties of the material is realized by bleaching, the strength properties being enhanced due to the removal of the lignin.

Compared with the conventional acid bisulfite decomposition using liquors containing the usual amount of free SO<sub>2</sub> at a highly acid pH (ca. 2-3), semi-chemical cellulose pulp with even better strength properties is obtained when the acid is buffered to a higher initial pH=about 4-6 and a temperature of about 125-130° is employed. In carrying out the new process according to the invention, any suitable acid, e. g. bisulfite liquor, can be used in making up the cooking acid. The acid should be diluted and gassed-up to such extent that by addition of the calculated amount of dilute buffer solution, e. g. caustic soda solution, the particular SO<sub>2</sub>-concentration desired is obtained. The requisite caustic soda or the like for raising the pH value can not be calculated stoichiometrically but must be determined in each instance. The character of the complex builder is of essential influence on the amount of buffer solution which has to be added. It appears that the addition of a certain amount of caustic soda solution for buffering reaches a maximum pH value in the presence of the complex builder and that, upon further additions, a drop in pH takes place which is accompanied by a strong clouding of the solution.

After adjustment of the desired pH value, the cooking liquid is heated up to the temperature of 105-120°, depending upon the starting material, necessary for the sulfonation. The per se known impregnation, and formation of the lignin sulfonic acid, takes place at these temperatures within about 3-7 hours, depending upon the starting material. An increase in temperature of 10-20°, above the foregoing temperature causes a hydrolytic splitting of the lignin sulfonic acid of the lignin sulfonic acid-cellulose compounds to take place in 3-5 hours, so that a loosening up of the fiber bundles takes place. The SO<sub>2</sub>-content of the cooking acid drops during the impregnation and cooking.

By degasification of the cooking lignin upon termination of the cooking, a part of the unconsumed SO<sub>2</sub> can be recovered from the spent liquor.

The semi-chemical cellulose pulp shreds obtained by the decomposition can be defibrillated into individual fibers in a known manner with the usual defibrillating devices, such as disk mills or the like, to obtain the resultant fibers which are of light color, somewhat like that of unbleached conventional sulfite cellulose. The waste liquors can be recovered and used for the production of yeast.

With the same process of the invention, the strength properties depend on the pH as shown by the following two examples for which two beech semi-chemical pulps were employed and having the same cellulose yield:

TABLE IV

| Yield.....                               | 70%                   | 68%   | 79%   | 81%   | 70%          | 68%   | 79% | 81%   |
|------------------------------------------|-----------------------|-------|-------|-------|--------------|-------|-----|-------|
| Starting pH.....                         | 4.3                   | 5.0   | 4.4   | 5.7   | 4.3          | 5.0   | 4.4 | 5.7   |
| Grinding Degree—Degrees Schopper-Riegler | breaking length in m. |       |       |       | rubbing test |       |     |       |
| 20.....                                  | 3,700                 | 4,700 | 3,300 | 4,500 | 20           | 120   | 10  | 80    |
| 40.....                                  | 5,500                 | 6,300 | 5,000 | 6,100 | 120          | 600   | 40  | 280   |
| 60.....                                  | 5,900                 | 6,900 | 5,700 | 7,000 | 320          | 1,360 | 90  | 520   |
| 80.....                                  | 6,700                 | 7,800 | 6,700 | 8,300 | 1,200        | 2,320 | 400 | 1,120 |

## EXAMPLE 1

50 kg. of birch wood chips with a moisture content of 11% are charged into a rotating cooker with 240 liters of decomposing liquor. In accordance with the inven-

tion, use is made of a cooking acid with a pH of 4.3, having a total SO<sub>2</sub>-content of 1.57%, 46% of the SO<sub>2</sub> being bound to CaO, and 27% being buffered by NH<sub>3</sub>. The pH value of 4.3 is realized by the addition of 50 mg./liter of Calgon, Na<sub>5</sub>P<sub>3</sub>O<sub>10</sub>, a water softening agent containing sodium hexametaphosphate as the main constituent.

The cooking temperature is raised to 105° C. in 1 hour, maintained at this temperature for 6 hours, heated 1 hour at 115° C. and 3 additional hours at 115° C. After raising the temperature to 125° for 4 hours, as is necessary for the decomposition of the lignosulfonic acid, the cooking is ended.

The pH-value drops during the cooking to about 2.9-3.0. Compared to an unbuffered cooking acid, this represents a terminal pH value which is higher by one pH unit. This difference of one unit shows up greatly at elevated temperature so that, due to weaker hydrolytic treatment much better yields and strength properties are obtained.

The obtained semi-chemical cellulose pulp shreds are defibrillated in known manner in a disk mill.

The yields amount to 82% relative to the starting wood.

Analytical date of the unbleached material follows:

|                                                  |      |
|--------------------------------------------------|------|
| Degree of decomposition (accdg. to Sieber) ----- | 95   |
| Lignin (Halse), percent -----                    | 12.6 |
| Cu-viscosity, cp. -----                          | 300  |
| Alpha-cellulose, percent -----                   | 76   |
| Pentosan, percent -----                          | 18.5 |

After a grinding in the Jokro mill, standard strength values are obtained:

| 35      | Degree of Grinding—Degrees Schopper-Riegler | Breaking Length, cm. | Folding Number | Breaking Pressure, kg./sq. cm. |
|---------|---------------------------------------------|----------------------|----------------|--------------------------------|
| 13..... | 2.8                                         | 5                    | 1.0            |                                |
| 28..... | 7.7                                         | 800                  | 4.1            |                                |
| 37..... | 8.6                                         | 1,500                | 4.5            |                                |
| 70..... | 8.5                                         | 1,400                | 4.6            |                                |
| 90..... | 8.4                                         | 600                  | 4.0            |                                |

The measurements in Example 1 and all of the remaining examples were obtained as follows:

The degree of whiteness in percent GE was measured with an American "General Electric Brightness Tester," which is described in TAPPI T217 m-48.

The degree of grinding fineness was determined with a Schopper-Riegler (SR) degree of fineness tester.

Tearing length, fold number and breaking pressure were determined by the method of "Verein der Zellstoff- und Papier-Chemiker und Ingenieure," a technical publication for cellulose strength testing, pages 101-103, Otto Elsner Verlag, Berlin.

The degree of decomposition and the copper viscosity were carried out according to the book by Dr. Rud. Sieber, "Die Chemisch-Technischen Untersuchungs-Methoden

der Zellstoff- und Papierindustrie, Springer-Verlag, Berlin, 1943," which is conventionally used in Germany, and the degree of decomposition being carried out according to the Sieber book, page 340, "determination of the

chlorine consumption number according to Sieber (Sieber number);

Copper viscosity was determined according to the Kung-Modified Method of the Technical Association of the Pulp and Paper Industry, Sieber book, page 514 et seq.;

Alpha cellulose was determined according to TAPPI T201 m-46.

EXAMPLE 2

In a jacketed cellulose digester, a cooking acid which contains 1.6% total  $\text{SO}_2$  and 0.6% CaO is added to beechwood chips. The pH value is adjusted to 4.6 by buffering with 0.5% NaOH in the presence of 50 mg./liter of nitrilotriacetic acid  $\text{N}(\text{CH}_2\text{CO}_2\text{H})_3$ . After impregnation for 6 hours at 105°, final cooking is carried out in 4 hours at 128° C. The  $\text{SO}_2$ -content of the cooking liquid is about 0.5% at the end of the cooking.

The waste liquor contains 11% reducing substance.

The semi-chemical cellulose pulp, obtained in a yield of 76%, determined according to standard methods, has the following strength properties:

| Degree of Grinding—°S. R. | Tearing Length, km. | Folding Number | Breaking Pressure, kg./sq. cm. |
|---------------------------|---------------------|----------------|--------------------------------|
| 15                        | 2.2                 |                | 0.73                           |
| 30                        | 5.6                 | 1              | 2.6                            |
| 50                        | 6.4                 | 350            | 3.0                            |
| 70                        | 7.4                 | 600            | 3.5                            |
| 85                        | 8.3                 | 1,600          | 4.0                            |

The strength properties of the product, which is prepared with a cooking acid of the same  $\text{SO}_2$ -concentration but without buffering according to the invention, are essentially lower. The maximum tear length at 85° S. R. is only 6.5 km., the fold numbers run about 350 and the breaking pressure is 3.5 kg./cm.<sup>2</sup>.

By stage bleaching, with an amount of chlorine of 14%, a bleached cellulose with a degree of whiteness of 86% G. E. is obtained in a yield of 64% calculated relative to the wood. The strength properties are further improved by the removal of lignin and have the following values:

| Degree of Grinding—°S. R. | Tearing Length, km. | Folding Number | Breaking Pressure, kg./sq. cm. |
|---------------------------|---------------------|----------------|--------------------------------|
| 20                        | 3.2                 | 20             | 1.5                            |
| 25                        | 5.9                 | 500            | 3.6                            |
| 40                        | 7.9                 | 2,000          | 4.5                            |
| 67                        | 8.7                 | 4,800          | 5.6                            |
| 85                        | 9.3                 | 5,500          | 5.7                            |

EXAMPLE 3

Pine wood chips are covered in a cooker with a cooking liquid which contains 2.2% total  $\text{SO}_2$ , 0.56% CaO and 0.5% NaOH. The pH value is adjusted to 4.2 by the addition of caustic soda solution in the presence of a tripolyphosphate of the formula,  $\text{H}_5\text{P}_3\text{O}_{10}$ . In the usual way, the initial temperature is maintained constant for 4 hours below 105°. After a 3-hour intermediate temperature of 115°, decomposition of the lignin sulfonic acid is achieved by a 6-hour cooking at 135°. The  $\text{SO}_2$ -content of the cooking acid drops, during the cooking, to 0.4%. Upon completion of the cooking, the pH value is 3.4. A 77% yield is obtained of a light-colored pine semi-chemical cellulose pulp, which is easily defibered, and which has a degree of decomposition (according to Sieber) of 97 and a Cu-viscosity of 250 cp.

The strength properties determined according to standard methods are the following:

| Degree of Grinding—°S. R. | Tearing Length, km. | Folding Number | Breaking Pressure, kg./cm. <sup>2</sup> |
|---------------------------|---------------------|----------------|-----------------------------------------|
| 13                        | 4.9                 | 400            | 2.6                                     |
| 20                        | 8.8                 | 1,700          | 4.9                                     |
| 42                        | 9.4                 | 2,200          | 5.5                                     |
| 69                        | 10.5                | 2,900          | 5.5                                     |
| 87                        | 10.4                | 5,000          | 6.3                                     |

The achieved strengths are very good; they are not equaled even by the usual good kraft materials.

The bleachability of the semi-chemical cellulose pulp is good. A yield of 59% relative to the wood is obtained. 5 There are a degree of whiteness of 86%, a maximum tear length of 9000 m. and a folding number of 6000 in the product.

EXAMPLE 4

10 A ten-fold quantity of cooking acid, which contains 1.3%  $\text{SO}_2$ , 0.64% CaO, 0.3% NaOH and 0.005% of a sodium tripolyphosphate of the formula,  $\text{Na}_5\text{P}_3\text{O}_{10}$ , is added to an unsorted mixture of comminuted wheat straw in a cooker provided with a circulating pump. After a pre-cooking period of 3 hours and a cooking period of 7 hours at 123°, a readily defibered product is obtained in a yield of 81%. Of the added  $\text{SO}_2$ , 12% can be recovered by degasification following the cooking.

EXAMPLE 5

20 In a jacketed cellulose cooker provided with a recycler, beechwood chips are treated with a magnesium bisulfite acid. The amount of  $\text{SO}_2$  used is 88 kg. per ton of absolutely dry wood. The pH value of the cooking acid, employed in the proportion of 5 cubic meters per ton of wood, was raised to a pH of 6.2 by the addition of dilute caustic soda solution in the presence of 50 mg. per liter of sodium hexametaphosphate of the formula  $(\text{NaPO}_3)_6$ .

25 After an impregnation stage at 105° C., the cooking takes place for a period of 4 hours at 152° C. maximum temperature. There is produced a semi-chemical cellulose pulp in a yield of 72%, which semi-chemical cellulose pulp can be defibered in normal manner in a disk mill.

30 35 The thus obtained cellulose is distinguished by an especially high pliability for beechwood as is shown by the very high folding number of 2000 at a degree of grinding of 83° Schopper-Riegler. The tear length, at this degree of grinding, is 8000 meters. The semi-chemical cellulose pulp can be bleached in a four-stage bleach with a total of 12.5% chlorine, relative to the material, to a whiteness degree of 83% GE.

EXAMPLE 6

45 45 Wheat straw is treated in a rotary cooker with a sevenfold quantity of an ammonium bisulfite cooking acid which contains 1.56% total  $\text{SO}_2$ ; 0.88%  $\text{SO}_2$  being bound to ammonia. The pH value of this solution is 5.1.

50 55 After a cooking period of 11 hours at 130°, semi-chemical cellulose pulp is obtained which can be readily defibrillated and can be bleached with 9.5% chlorine. The degree of whiteness of the bleached material, obtained in a yield of 58%, is 85% degree-units. The strength properties of the unbleached semi-chemical cellulose pulp are, for a degree of grinding of 83 Schopper-Riegler, 7500 meters tear length and 3500 double folds.

EXAMPLE 7

60 65 Beechwood chips are treated in a cooker with a sodium bisulfite cooking acid having an  $\text{SO}_2$ -content of 1.6%. The quantity of cooking acid is adjusted that 4-5 cubic meters of acid per ton of wood is used. The NaOH-bound amount of  $\text{SO}_2$  is of such magnitude that a pH value of 5.8 prevails. After a precooking and impregnating period of 8 hours and a following cooking period of 8 hours at 135°, a 73% yield of easily defibrillated product is obtained.

EXAMPLE 8

70 75 Pine wood chips are covered in a cooker with a cooking liquid which contains 2.2% total  $\text{SO}_2$ , 0.5% CaO and 0.5% NaOH. The pH value is adjusted to 4.2 by the addition of caustic soda solution in the presence of 0.4% methylamine in solution. In the usual way, the initial temperature is maintained constant for 4 hours below 105°. After a 3-hour intermediate temperature of

115°, decomposition of the lignin sulfonic acid is achieved by a 6-hour cooking at 135°. The SO<sub>2</sub>-content of the cooking acid drops, during the cooking, to 0.4%. Upon completion of the cooking, the pH value is 3.4. A 77% yield is obtained of a light-colored pine semi-chemical cellulose pulp, which is easily defibered, and which has a degree of decomposition (according to Sieber) of 97 and a Cu-viscosity of 250 cp.

The achieved strengths are very good; they are not equalled even by the usual good kraft materials.

The bleachability of the semi-chemical cellulose pulp is good.

In each of the examples above, any of the polyphosphates mentioned may be used interchangeably in appropriate equivalent quantities with the pyrophosphates, imidoacetic acid and nitrilotriacetic acid without any change in the process conducted and product obtained.

Likewise the imidoacetic acid, nitrilotriacetic acid and pyrophosphates may be used interchangeably with each other and with the polyphosphates, without change in the process conducted and product obtained.

Having thus disclosed the invention, what is claimed is:

1. Process for the preparation of semi-chemical cellulose which comprises treating cellulose-containing raw materials obtained from foliaceous trees, coniferous trees and annual plants with buffered bisulfite cooking solutions consisting of aqueous sulfur dioxide containing about 1.4-3.0% sulfur dioxide and a base selected from the group consisting of the hydroxides of calcium, magnesium, sodium, and ammonium, in an amount, depending upon the base and cellulose raw material employed, to provide an initial pH value of 3.5-6, cooking with said solution in the presence of a buffer selected from the group consisting of alkali metal hexametaphosphates, tri-polyphosphates, polyphosphates and pyrophosphates at a

reaction temperature of 115-140° C., to repress the excessive hydrolytic decomposition of the cellulose and to remove a substantial amount of the lignin binding the cellulose fibers in the middle lamallae, and thereafter mechanically subdividing the product into individual fibers.

2. A process as in claim 1 wherein the base is calcium hydroxide and the initial pH is 4.5 at a reaction temperature of 125-130° C.

3. A process as in claim 1 wherein the base is magnesium hydroxide and the initial pH is 5-6.

#### References Cited in the file of this patent

##### UNITED STATES PATENTS

|           |            |               |
|-----------|------------|---------------|
| 1,244,525 | Marusawa   | Oct. 30, 1917 |
| 1,566,118 | Rawling    | Dec. 15, 1925 |
| 1,792,510 | Richter    | Feb. 17, 1931 |
| 1,859,848 | Rue et al. | May 24, 1932  |
| 1,891,337 | Seaman     | Dec. 20, 1932 |
| 2,019,598 | Dreyfus    | Nov. 5, 1935  |
| 2,564,028 | Parrett    | Aug. 14, 1951 |

##### FOREIGN PATENTS

|         |               |               |
|---------|---------------|---------------|
| 384,455 | Great Britain | Dec. 8, 1932  |
| 496,841 | Belgium       | July 31, 1950 |

##### OTHER REFERENCES

Richter, Chemical Abstracts 35, 3439.  
 Benjamin, Com. of Australia, Council of Sci. and Ind. Res. Bull. 37, page 76 (1928), Cook 156.  
 Manufacture of Pulp and Paper, 3d ed., vol. III, Sec. 4, pp. 1, 2, 59 (1937), published by McGraw-Hill, N. Y.  
 Yorston, Canada Dept. of Mines and Resources DFS-Bull. 97, pp. 21, 33, 34, 53 and 80 (1942).